

# UNITED STATES PATENT OFFICE.

ROBERT ABBOTT HADFIELD, OF SHEFFIELD, ENGLAND.

## PROCESS OF IMPROVING THE MAGNETIC QUALITIES OF IRON-SILICON-ALUMINIUM ALLOYS.

No. 836,497.

Specification of Letters Patent.

Patented Nov. 20, 1906.

Application filed August 21, 1906. Serial No. 331,421.

*To all whom it may concern:*

Be it known that I, ROBERT ABBOTT HADFIELD, a subject of the King of Great Britain, and a resident of Sheffield, England, have invented a certain new and useful Improvement in Processes of Improving the Magnetic Qualities of Iron-Silicon-Aluminium Alloys, of which the following is a specification.

- 10 In another application for Letters Patent, Serial No. 324,894, filed July 5, 1906, I have described and claimed an alloy of iron with silicon in such proportion as to reduce the total magnetic and electric losses in the mixture (when such alloy is used for ballast-coils, transformer-plates, or like electric apparatus) to which alloy aluminium is added in order to improve the solidity and homogeneity thereof when in cast or molded condition. 15 In order to effect the best reduction of the said magnetic and electric losses, a heat treatment of said alloy is necessary.

20 My present invention is a process of heat treatment applied to the aforesaid iron-silicon-aluminium alloy for the purpose stated.

25 In carrying my invention into effect I first prepare an alloy of iron and silicon in molten state and add aluminium or other powerful deoxidizer, cast the mass into ingots, and 30 convert the ingots into desired shapes and thicknesses by appropriate means. An example of such an alloy may contain iron and silicon in proportion of from one to five per cent. and aluminium in proportion less than 35 one per cent., as set forth in my aforesaid application. I then heat said alloy to a temperature above a critical point (hereinafter defined) and then cool said alloy slowly. When said alloy is subjected to progressive 40 temperature variations (below fusion) from 600° centigrade upward, it undergoes at a certain temperature point an apparent molecular change, and on further alteration of temperature another point ensues at which 45 another molecular change occurs. The term "critical point" herein used means the point of higher temperature of the two above noted and corresponds and approximates to

the 900°-centigrade point in the case of pure iron, which is the lower limit of its so-called "gamma" state. This gamma state is definitely shown, for example, in ordinary carbon-steels when heated. A diagram accurately illustrating this point is given by Messrs. Arnold and McWilliam in their paper on the thermal transformations of carbon-steels published in the *Journal of the Iron and Steel Institute*, 1905, Vol. 2. Diagram 2 in this paper shows the critical point for a certain carbon-steel at about 870° centigrade. In practice I have subjected my said alloy to a temperature of about 1,050° centigrade and then cooled the same slowly at the approximate rate of 10° centigrade per hour. The alloy should be low in carbon and manganese—say carbon under about .12 per cent. and manganese under about .12 per cent. For certain purposes, if desired, the material as cast may be used, being suitably treated in the same manner as the forged or rolled material.

I claim—

1. The process of increasing the magnetic permeability and electric resistance and reducing the hysteresis action of an iron-silicon-aluminium alloy, low in carbon and manganese, which consists in heating said alloy to a temperature above its critical point, and then cooling.

2. The process of increasing the magnetic permeability and electric resistance and reducing the hysteresis action and also of solidifying the structure of an iron-silicon alloy, low in carbon and manganese, which consists in melting iron and silicon, adding aluminium, casting into ingot form, converting the ingot into desired shapes by appropriate means, then heating said alloy to a temperature above the critical point of said alloy and finally cooling.

In testimony whereof I have signed my name hereto in the presence of two witnesses.

ROBERT ABBOTT HADFIELD.

Witnesses:

WILLIAM CROSS,

WILLIAM CRAWLEY.